# EUROPEAN PATENT SPECIFICATION

(11) **EP 0 432 946 B1**
(45) Date of publication and mention of the grant of the patent: **23.04.1997**
(21) Application number: 90313047.4
(22) Date of filing: 30.11.1990
(51) Int. Cl.: G03G 9/097

(54) **Charge control resin particles for an electrophotographic toner and a method of manufacturing the same**
Ladungskontrollharzteilchen für einen elektrophotographischen Toner und Verfahren zu ihrer Herstellung
Particules de résine de contrôle de charge pour un toner électrophotographique et leur procédé de préparation

(30) Priority: 30.11.1989 JP 312481/89
(43) Date of publication of application: 19.06.1991
(73) Proprietor: MITA INDUSTRIAL CO., LTD., Osaka 540 (JP)
(72) Inventor: Shimoyama, Hiroshi, Osaka-shi, Osaka (JP); Tokuno, Toshiro, Takarazuka-shi, Hyogo-ken (JP)
(74) Representative: Cheyne, John Robert Alexander Mackenzie

(56) References cited:
- EP-A- 0 330 287
- GB-A- 2 070 036
- GB-A- 2 083 051
- PATENT ABSTRACTS OF JAPAN vol. 11, no. 253 (P-606)(2700) 18 August 1987, & JP-A-62 59964 (RICOH CO.,LTD.) 16 March 1987,

## Description

The present invention relates to resin particles having a specific size and size distribution for use as electric charge control agents in toner for developing an electrostatic image used in electrophotography, and to a dispersion polymerization method of manufacturing the same.

Generally, the toner for developing electrostatic images used in the field of electrophotography or the like is formed from resin particles of 5 to 20 µm in size consisting of colorants, charge control agents, etc. dispersed in binding resin particles. The charge control agents used to confer triboelectrification ability on the resin particles include nigrosine, monoazo dyes, or metallic complexes of salicylic acid or naphthoic acid, etc. However, since most of these charge control agents lack compatibility with binding resins, the charge control agents become dispersed unevenly in the resin particles, preventing uniform conferring of frictional chargeability. In view of such difficulty, there has been proposed a method wherein charge control resins having polar functional groups are mixed into binding resins to confer frictional chargeability to the toner. For such charge control resins, compatibility with binding resins is required, and generally, a copolymer is used which consists of a water-soluble monomer having a polar group, such as acrylonitrile and styrene sulfonic acid sodium salt., and an oil-soluble monomer capable of forming a polymer having compatibility with the binding resins. In this connection, EP-A-0 330 287 discloses a toner for developing statically charged images which comprises a copolymer comprising a water soluble monomer having a group -SO₃X in which X stands for hydrogen, sodium, potassium or calcium and an oil-soluble monomer. The copolymer is incorporated into a polymerizable composition comprising a polymerizable monomer, an initiator and a colorant. Dispersion stabilizers are used for suspension polymerization of toner particles. Fine polymer particles having a size smaller than 5 µm and 8 µm are disclosed.

Bulk polymerization, suspension polymerization, solution polymerization, emulsion polymerization, and dispersion polymerization are used for manufacturing the charge control resins. Since the compatibility is generally low between a water-soluble monomer having a polar group and an oil-soluble monomer, a uniform polymer system cannot be formed in bulk polymerization or in suspension polymerization, the resulting copolymer having a large quantity of monomeric units having a polar group and thus lacking compatibility with binding resins. In solution polymerization, it is possible to make the polymer system uniform before polymerization by choosing an appropriate solvent, but as the polymerization progresses, the polymer precipitates, making the composition of the final copolymer non-uniform. In emulsion polymerization, it is possible to control the compositions of the monomers in the copolymer, but since the molecular weight of the copolymer is very high, the compatibility with binding resins is low. Furthermore, in emulsion polymerization, the problem is that the size of the obtained particles is small, thus making it difficult to precipitate the particles. In dispersion polymerization, uniform polymerization is possible, but the size distribution of the obtained particles is broad and the molecular weight tends to become high, thus leaving room for improvement.

According to the present invention, there is provided electrophotographic toner charge control resin particles which are spheroidal and are composed mainly of a copolymer formed from at least one water-soluble monomer having an anionic group of sulfonic, carboxylic or phosphoric type and at least one oil-soluble monomer, wherein the copolymer has a weight-average molecular weight of 3,000 to 50,000, the resin particles being formed by dispersion polymerisation and having a volume median size of 3µm to 10µm and the ratio D₂₅/D₇₅ of 25 volume percent integrated diameter D₂₅ to the 75 volume percent integrated diameter D₇₅ within the range of 1 to 1.4.

It is preferred that the anionic group be a sulfonic group or an alkali metal salt thereof. A preferred monomer is then styrene sulfonic acid sodium salt.

It is further preferred that the oil-soluble monomer comprises both styrene and an acrylic monomer.

The ratio of the water-soluble monomer to the oil-soluble monomer forming the copolymer is preferably in the range from 70:30 to 99:1 by weight.

The present invention also provides a dispersion polymerization method for manufacturing electrophotographic toner charge control resin particles as claimed in claim 1, wherein at least one water-soluble monomer having an anionic group of sulfonic, carboxylic or phosphoric type and at least one oil-soluble monomer are dispersed and polymerized in an aqueous medium containing water and a water-miscible organic solvent in the presence of a dispersion stabilizer and a chain transfer agent and the resulting copolymer consisting of the water-soluble monomer and the oil-soluble monomer is collected in the form of particles, the polymerization including the steps of: forming a nucleus by reaction of the oil-soluble monomer and the water-soluble monomer; and growing the thus formed nucleus, the temperature being higher in the nucleus growing step than in the nucleus forming step.

In a preferred embodiment, the mixing ratio of the water and the water-miscible organic solvent in the aqueous medium is in the range from 40:60 to 5:95 by weight.

In another preferred embodiment, the temperature is 60 to 80°C in the nucleus forming step and 70 to 90°C in the nucleus growing step.

Thus, the invention described herein makes possible one or more of the objectives of (1) providing charge control resin particles having a narrow size distribution and formed from a resin having a relatively low molecular weight; (2) providing charge control resin particles comprising a polymer with a low molecular weight and having a large particle size in the dispersion liquid; (3) providing charge control resin particles having good compatibility with a binding resin or with a monomer forming the binding resin and therefore capable of forming toner with the charge control resin uniformly dispersed in the binding resin; (4) providing charge control resin particles having uniform chargeability over the entire toner particles and therefore capable of forming toner having excellent charge characteristics; and (5) providing a method capable of readily producing the charge control resin particles having the above-mentioned excellent characteristics.

In the polymer system of the present invention, reaction progresses in solution polymerization in the early stage of polymerization, to form a copolymer comprising monomers having a composition ratio that matches their reactivity ratio. As the polymerization further progresses, the copolymer tries to precipitate, but since a dispersion stabilizer exists in the polymer system, it is believed that some of copolymers combine to form a relatively stable nucleus (dispersed particle). It is believed that since this nucleus is a copolymer formed from an oil-soluble monomer and a water-soluble monomer, the unreacted oil-soluble monomer and water-soluble monomer in the continuous phase are simultaneously absorbed and the polymerization progresses after formation of the nucleus, thus forming a copolymer having a relatively uniform composition. Particularly, when styrene and an acrylic monomer are used simultaneously as the oil-soluble monomer, the particle size is relatively large in the dispersion liquid and particles are readily precipitated therefrom. Furthermore, by using these monomers, the copolymer forming the particles has a relatively low molecular weight.

In the present invention, since a chain transfer agent exists in the reactive system, the molecular weight of the copolymer is kept low.

It is believed that since the temperature is relatively low in the nucleus forming step and relatively high in the nucleus growing step, stable formation of the nucleus is facilitated and the incorporation of the monomers into the nucleus and the polymerization reaction are effectively performed, thus forming charge control resin particles having a low molecular weight and a uniform size distribution.

The charge control resin particles have a large volume median size of 3 µm to 10 µm, and therefore, the handling thereof, including separation from a mixture liquid, is facilitated. Also, since they are formed from a low molecular weight copolymer having a weight-average molecular weight of 3,000 to 50,000, the resin particles are evenly and uniformly dissolved within a binding resin such as a styrene copolymer or in monomers forming the binding resin. Furthermore, since the degree of dispersion expressed by the ratio D₂₅/D₇₅ of the 25 volume percent integrated diameter D₂₅ to the 75 volume percent integrated diameter D₇₅ of the resin particles is within the range of 1 to 1.4 and the particle size distribution is sharp, the toner particles with the charge control resin particles dispersed therein are provided with uniform chargeability over the entire particles and exhibit excellent charge characteristics. Also, when producing toner by suspension polymerization using the charge control resin particles, since the viscosity of suspended oil does not increase and the polarity of the oil is uniform, toner particles having an extremely sharp size distribution can be obtained.

The oil-soluble monomer used for the present invention is a monomer capable of forming a polymer having a good compatibility with binding resins. Hydrophobic monomers such as vinyl aromatic monomers, acrylic monomers such as vinyl ester monomer, vinyl ether monomer, and olefinic monomers are used. The vinyl aromatic monomers include, for example, styrene, α-methylstyrene, vinyltoluene, α-chlorostyrene, o-, m-, p-chlorostyrene, p-ethylstyrene, divinylbenzene. The acrylic monomers include, for example, methyl acrylate, ethyl acrylate, butyl acrylate, 2-ethylhexylacrylate, cyclohexyl acrylate, phenyl acrylate, methyl methacrylate, hexyl methacrylate, 2-ethylhexyl methacrylate, β-hydroxyethyl acrylate, γ-hydroxypropyl acrylate, δ-hydroxybutyl acrylate, β-hydroxyethyl methacrylate, and ethyleneglycol dimethacrylate. The vinyl ester monomers include, for example, vinyl formate, vinyl acetate, and vinyl propionate. The vinyl ether monomers include, for example, vinyl-n-butyl ether, vinyl phenyl ether, and vinyl cyclohexyl ether. The olefinic monomers include, for example, ethylene, propylene, isobutylene, butene-1, pentene-1, and 4-methylpentene-1. Two or more of these monomers can be used simultaneously.

The water-soluble monomer used for the present invention has an anionic group of sulfonic, carboxylic or phosphoric type. These acid radicals may be either in the form of salts such as sodium salt and other alkali metal salts, ammonium salt, amine salt, etc., or in the form of free acids. Monomers having a sulfonic group or its alkali metal salt are particularly desirable. Such monomers include, for example, styrenesulfonic acid, styrenesulfonic acid sodium salt, 2-acrylamide-2-methylpropanesulfonic acid, 2-phosphoxypropylmethacrylate, 2-phosphoxyethylmethacrylate, 3-chloro-2-phosphoxypropylmethacrylate, acrylic acid, methacrylic acid, fumaric acid, crotonic acid, tetrahydroterephthalic acid, itaconic acid, maleic acid, etc. The styrenesulfonic acid sodium salt is most preferable.

The composition al ratio of the water-soluble monomer to the oil-soluble monomer should be determined in such a manner as to obtain good compatibility with the binding resin and good charge characteristics. Generally the ratio should be in the range of 70: 30 to 99: 1, and preferably 80: 20 to 98 : 2, by weight.

With an oil-soluble monomer comprising styrene and an acrylic monomer, the mixing ratio of styrene and acrylic monomer is preferably in the range of 10 : 0.1 to 10: 3, by weight. If the amount of an acrylic monomer exceeds the above range, the particles tend to adhere, thereby causing difficulty in handling thereof. Moreover, other radical polymeric monomers can be included as needed. The amount of these monomers used is preferably 20 percent by weight or less.

If the water-soluble monomer is styrenesulfonic acid sodium salt the mixing ratio of the oil-soluble monomer to styrenesulfonic acid sodium salt is preferably in the range of 70: 30 to 99: 1, by weight.

In the present invention, known chain transfer agents are used which include, for example, octyl thioglycolate.

Polymeric dispersion stabilizers are desirable for use as the dispersion stabilizer, and include, for example, polyacrylic acid, salts of polyacrylic acid, polymethacrylic acid, salts of polymethacrylic acid, (meth)acrylic acid-(meth)acrylic acid ester copolymer, acrylic acid-vinylether copolymer, methacrylic acid styrene copolymer, carboxylmethyl cellulose, polyethylene oxide, polyacrylamide, methyl cellulose, ethyl cellulose, hydroxyethyl cellulose polyvinyl alcohol, etc. Nonionic or anionic surfactant may also be used. The amount of the dispersion stabilizer added is preferably 1 to 20 percent by weight, with respect to the monomers.

The water-miscible organic solvents which can be used include, for example, lower alcohols such as methanol, ethanol, isopropanol, etc.; ketones such as acetone, methyl ethyl ketone, methyl bytyl ketone, etc.; ethers such as tetrahydrofuran, dioxane etc.; esters such as ethyl acetate, etc.; and amides such as dimethylformamide, etc.

The mixing ratio of the water to the water-miscible organic solvent depends on the kind of the monomer and the kind of the organic solvent. Generally the ratio should be within the range of 40: 60 to 5: 95 by weight, and preferably within the range of 30: 70 to 10: 90 by weight. The composition ratio is preferably determined so as to have a uniform solution phase within this range. The amount of the medium used is 0.5 to 50 times by weight with respect to a monomer, particularly 5 to 25 times by weight being preferable.

When practicing the method of the present invention, the charge control resin particles may be manufactured, for example, in the following manner. The oil-soluble monomer, water-soluble monomer, dispersion stabilizer, and if necessary, a polymerization initiator, are dissolved in a solution of water and a water-miscible organic solvent, and the chain transfer agent is further added. After stirring the mixture for 0.5 to 4 hours at a temperature of 60 to 80°C, the temperature of the mixture is raised to 70 to 90°C and the liquid is then stirred for 2 to 20 hours. At this time, it is desirable that this process is conducted in the presence of an inert gas to suppress polymerization termination by oxygen. The resulting polymer is filtered, washed with water or other suitable solvent as necessary, and dried to obtain the desired resin particles.

Any hydrophobic polymerization initiator is used as the polymerization initiator. For such initiators, azo compounds such as azobisisobutyronitrile, etc. and peroxides such as cumene hydroperoxide, di-t-butylperoxide, benzoyl peroxide, lauroyl peroxide, etc. are used. The mixing ratio of the initiator is not specifically limited, but should generally be 0.1 to 20 percent by weight with respect to the monomer. Instead of using such initiators, the polymerization can be initiated by using gamma rays or an accelerated electron beam. Alternatively, the polymerization may be initiated by using photosensitizers in combination with ultraviolet rays.

The thus obtained charge control resin particles have a relatively large average size of 3 to 10 µm in a dispersion liquid , so the precipitation thereof from the mixture is facilitated. The particles are composed of polymers having a weight of 3,000 to 50,000. Since the molecular weight is relatively low, the resin particles have good compatibility with the binding resin such as a styrene copolymer or with monomers forming the binding resin, and therefore, a toner with the charge control resin particles uniformly dispersed in the binding resin can be readily obtained. Furthermore, since the ratio D₂₅/D₇₅ of the 25 volume percent integrated diameter D₂₅ to the 75 volume percent integrated diameter D₇₅ is within the range of 1 to 1.4 and the particle size distribution is extremely monodisperse, the toner particles with the charge control resin particles dispersed therein are provided with uniform chargeability over the entire particles and exhibit excellent charge characteristics. According to the present invention, charge control resin particles having the above-mentioned excellent characteristics can be readily manufactured.

The following Examples illustrate the present invention.

### Example 1

Ten grams of polyacrylic acid were dissolved in a solution consisting of 675 g of isopropyl alcohol and 225 g of water, to which 90 g of styrene, 10 g of styrene sulfonic acid sodium salt, 5 g of octyl thioglycolate, and 7.5 g of azobisisobutyronitrile were added. The thus prepared liquid was placed in a 3-liter separable flask for 2 hours at 70°C while the liquid was being stirred in a 150 rpm stream of nitrogen, after which the temperature was raised to 80°C to perform a reaction for 10 hours, after which polymerization was completed. The obtained emulsion was observed under an optical microscope to note the formation of particles having a median size of about 6.0 µm. The ratio D₂₅/D₇₅ was 1.37 and a very sharp particle size distribution was noted. The weight-average molecular weight measured by gel permeation chromatography (GPC) was 1.18 x 10⁴. It was possible to collect 100% of the particles in a short time using a qualitative filter.

Ten parts by weight of the obtained styrene-styrenesulfonic acid sodium salt copolymer, 80 parts by weight of styrene-acrylic binder resin, and 10 parts by weight of carbon black were melted and kneaded, and the thus kneaded mixture was crushed and classified to obtain toner having an average particle size of 10 µm. The toner was mixed and stirred with ferrite carrier to prepare developer, which was then subjected to testing on a Mita Industrial Co., Ltd. Model DC-1205 copier to examine splashing and fogging of toner, changes in image density, etc. under high temperature and high humidity (35°C, RH85%) and low temperature and low humidity (10°C, RH45%) conditions. The result showed no problems. Further, the developer showed a high charge amount under the above conditions and also exhibited an extremely good charging-up. The charge distribution of the developer was measured on a toner charge distribution measuring instrument, which showed a sharp charge distribution with no uncharged or reverse charged toner whatsoever noted.

### Example 2

Ten grams of polymethacrylic acid were dissolved in a solution consisting of 700 g of isopropyl alcohol and 300 g of water, to which 90 g of styrene, 10 g of styrenesulfonic acid sodium, 3 g of octyl thioglycolate, and 7 g of 2,2'-azobis-2,4-dimethylvaleronitrile were added. The thus prepared liquid was placed in a 3-liter separable flask for 2 hours at 65°C while the liquid was being stirred in a 150 rpm stream of nitrogen, after which the temperature was raised to 75°C to perform a reaction for 10 hours, the polymerization being thus completed. The obtained emulsion was observed under an optical microscope to note the formation of particles having a size of about 4.2 µm. The ratio D₂₅/D₇₅ was 1.39, and the weight-average molecular weight measured on a GPC was 1.25 x 10⁴. It was possible to collect 100% of the particles in a short time using a qualitative filter.

Ten parts by weight of the obtained styrene-styrenesulfonic acid sodium salt copolymer, 80 parts by weight of n-butylacrylate, 10 parts by weight of grafted carbon black (MA-100, manufactured by Mitsubishi Kasei), 1.5 parts by weight of low molecular weight polypropylene (BISCALL 550P, manufactured by Sanyo Kasei), and 4 parts by weight of azobisisobutyronitrile were dissolved in this order in 60 parts by weight of styrene. At this time, the styrene-styrenesulfonic acid sodium salt copolymer was quickly dissolved, without flocculating, when charged into the styrene. The mixture was charged into an aqueous solution of 1.5% calcium phosphate (pH adjusted to 11 by sodium hydroxide) and dispersed for suspension therein using a TK-Homomixer (manufactured by Tokushu Kikou Kogyo), after which the mixture was polymerized for 5 hours while being stirred in a normal manner at 80°C in a stream of nitrogen. The thus produced particles were filtered, washed, and dried to obtain the toner. The thus obtained toner was spheroidal, had good flowability, and had sharp particle size and charge amount distributions. The toner was evaluated in the same manner as in Example 1, and yielded good results in all evaluations.

### Example 3

Ten grams of polyacrylic acid were dissolved in a solution consisting of 675 g of ethanol and 225 g of water, to which 90 g of styrene, 10 g of styrenesulfonic acid sodium, 5 g of octyl thioglycolate, and 10 g of benzoyl peroxide were added. The thus prepared liquid was placed in a 3-liter separable flask for 2 hours at 60°C while the liquid was being stirred in a 150 rpm stream of nitrogen, after which the temperature was raised to 80°C to perform a reaction for 10 hours, the polymerization being thus completed. The obtained emulsion was observed under an optical microscope to note the formation of particles having an average size of 4.6 µm. The ratio D₂₅/D₇₅ was 1.39, and the weight-average molecular weight measured on a GPC was 1.50 x 10⁴.

Toner was prepared in the same manner as in Example 2. The solubility of the styrene-styrenesulfonic sodium salt copolymer in the styrene was good. The obtained toner was evaluated in the same manner as in Example 1, and yielded good results in all evaluations.

### Comparative Example 1

The composition was the same as used was in Example 1 except that octyl thioglycolate the chain transfer agent and the polymerization was performed for 10 hours at a temperature of 70°C without raising the temperature during the polymerization.

The obtained styrene-styrenesulfonic sodium salt copolymer in the emulsion had an average particle size of 1.8 µm, thus forming particles of a small size. The ratio D₂₅/D₇₅ was 1.55 and the particle size distribution was broad. The weight-average molecular weight measured on a GPC was 10.88 x 10⁴. The copolymer had poor compatibility with monomers such as styrene, and it took time to dissolve the copolymer in the monomer.

### Comparative Example 2

The composition was the same as in Example 2 although the temperature was not raised during the polymerization but kept at 80°C throughout the polymerization.

The obtained styrene-styrenesulfonic sodium salt copolymer contained in the emulsion coarse agglomerate which accounted for 3% of the entire particles. The average size of the particles was 7.2 µm. The ratio D₂₅/D₇₅ was 1.70 and the particle size distribution was very broad. The weight-average molecular weight was 8.3 x 10⁴. Toner was prepared and evaluated in the same manner as in Example 2. When used, fogging was observed due to incomplete charging of toner particles, which was particularly noticeable under high temperature and high humidity conditions.

### Comparative Example 3

The composition was the same as that of Example 3 except that the temperature was not raised during the polymerization but was kept at 75°C throughout the polymerization.

The styrene-styrenesulfonic sodium salt copolymer particles contained in the emulsion particles were generally less than several µm, but there were particles of 10 to 20 µm size, showing a very broad particle size distribution.

## Claims

1. Electrophotographic toner Charge control resin particles which are spheroidal and are composed mainly of a copolymer formed from at least one water-soluble monomer having an anionic group of sulfonic, carboxylic or phosphoric type and at least one oil-soluble monomer, wherein the copolymer has a weight-average molecular weight of 3,000 to 50,000, the resin particles being formed by dispersion polymerization and having a volume median size of 3 µm to 10 µm, and the ratio D₂₅/D₇₅ of 25 volume percent integrated diameter D₂₅ to the 75 volume percent integrated diameter D₇₅ within the range of 1 to 1.4.

2. Charge control resin particles according to Claim I, wherein the anionic group is a sulfonic group or an alkali metal salt thereof.

3. Charge control resin particles according to Claim 2, wherein the water-soluble monomer is styrenesulfonic acid sodium salt.

4. Charge control resin particles according to any preceding claim, wherein the oil-soluble monomer comprises both styrene and an acrylic monomer.

5. Charge control resin particles according to any preceding claim, wherein the ratio of the water-soluble monomer to the oil-soluble monomer forming the copolymer is in the range from 70:30 to 99:1 by weight.

6. A dispersion polymerization method for manufacturing electrophotographic toner charge control resin particles as claimed in claim 1, wherein at least one water-soluble monomer having an anionic group of sulfonic, carboxylic or phosphoric type and at least one oil-soluble monomer are dispersed and polymerized in an aqueous medium containing water and a water-miscible organic solvent in the presence of a dispersion stabilizer and a chain transfer agent, and
the resulting copolymer consisting of the water-soluble monomer and the oil-soluble monomer is collected in the form of particles, the polymerization including the steps of:
forming a nucleus by reaction of the oil-soluble monomer and the water-soluble monomer; and
growing the thus formed nucleus;
the temperature being higher in the nucleus growing step than in the nucleus forming step.

7. A method for manufacturing charge control resin particles according to Claim 6, wherein the mixing ratio of the water and the water-miscible organic solvent in the aqueous medium is in the range of 40:60 to 5:95 by weight.

8. A method for manufacturing charge control resin particles according to claim 6 or 7, wherein the temperature is 60 to 80°C in the nucleus forming step and 70 to 90°C in the nucleus growing step.

## Patentansprüche

1. Harzteilchen zur Ladungskontrolle elektrophotographischer Toner, welche kugelförmig und im wesentlichen aus einem Copolymer zusammengesetzt sind, das aus mindestens einem wasserlöslichen Monomer mit einer anionischen Gruppe vom Sulfonsäure-, Carbonsäure- oder Phosphorsäuretyp und mindestens einem öllöslichen Monomer gebildet ist, wobei das Copolymer ein durchschnittliches Molekulargewicht (Gewichtsmittel) von 3000 bis 50 000 aufweist, die Harzteilchen durch Dispersionspolymerisation gebildet sind und eine Volumen-Mediangröße von 3 µm bis 10 µm aufweisen und das Verhältnis D₂₅/D₇₅ von integriertem 25 Vol.-% Durchmesser D₂₅ zu integriertem 75 Vol.-%-Durchmesser D₇₅ im Bereich von 1 bis 1,4 liegt.

2. Harzteilchen zur Ladungskontrolle nach Anspruch 1, in denen die anionische Gruppe eine Sulfonsäuregruppe oder deren Alkalimetallsalz ist.

3. Harzteilchen zur Ladungskontrolle nach Anspruch 2, in denen das wasserlösliche Monomer Styrolsulfonsäure-Natriumsalz ist.

4. Harzteilchen zur Ladungskontrolle nach einem der vorhergehenden Ansprüche, in denen das öllösliche Monomer sowohl Styrol als auch ein Acrylsäuremonomer umfaßt.

5. Harzteilchen zur Ladungskontrolle nach einem der vorhergehenden Ansprüche, in denen das Gewichtsverhältnis von dem das Copolymer bildenden wasserlöslichen Monomer zu öllöslichem Monomer im Bereich von 70:30 zu 99:1 liegt.

6. Dispersionspolymerisationsverfahren zur Herstellung von Harzteilchen zur Ladungskontrolle elektrophotographischer Toner gemäß Anspruch 1, bei dem mindestens ein wasserlösliches Monomer mit einer anionischen Gruppe vom Sulfonsäure-, Carbonsäure- oder Phosphorsäuretyp und mindestens ein öllösliches Monomer in einem wäßrigen Medium, das Wasser und ein mit Wasser mischbares organisches Lösungsmittel enthält, in Gegenwart eines Dispersionsstabilisierungsmittels und eines Kettenübertragungsreagenzes dispergiert und polymerisiert werden und
das resultierende, aus dem wasserlöslichen und dem öllöslichen Monomer bestehende Copolymer in Form von Partikeln gesammelt wird, wobei bei der Polymerisation:
durch Reaktion des öllöslichen und des wasserlöslichen Monomers ein Kern gebildet und
der so gebildete Kern wachsen gelassen wird,
wobei die Temperatur in der Kern-Wachstums-Stufe höher als in der kernbildenden Stufe ist.

7. Verfahren zur Herstellung von Harzteilchen zur Ladungskontrolle nach Anspruch 6, bei dem das Mischungs-Gewichtsverhältnis von Wasser und mit Wasser mischbarem organischen Lösungsmittel in dem wäßrigen Medium im Bereich von 40:60 bis 5:95 liegt.

8. Verfahren zur Herstellung von Harzteilchen zur Ladungskontrolle nach Anspruch 6 oder 7, bei dem die Temperatur in der kernbildenden Stufe 60 bis 80 °C und in der Kern-Wachstums-Stufe 70 bis 90 °C beträgt.

## Revendications

1. Particules de résine de régulation de charge pour toner électrophotographique qui sont sphéroïdales et composées principalement d'un copolymère formé par au moins un monomère hydrosoluble possédant un groupe anionique de type sulfonique, carboxylique ou phosphorique et au moins un monomère liposoluble, dans lesquelles le copolymère possède une masse moléculaire moyenne en masse de 3 000 à 50 000, les particules de résine étant formées par polymérisation en dispersion et ayant une taille moyenne en volume de 3 µm à 10 µm, et le rapport D₂₅/D₇₅ du diamètre intégré à 25 pourcent en volume D₂₅ au diamètre intégré à 75 pourcent en volume D₇₅ compris entre 1 et 1,4.

2. Particules de résine de régulation de charge selon la revendication 1, dans lesquelles le groupe anionique est un groupe sulfonique ou un sel alcalin de celui-ci.

3. Particules de résine de régulation de charge selon la revendication 2, dans lesquelles le monomère hydrosoluble est un sel sodique de l'acide styrènesulfonique.

4. Particules de résine de régulation de charge selon l'une des revendications précédentes, dans lesquelles le monomère liposoluble est constitué à la fois de styrène et d'un monomère acrylique.

5. Particules de résine de régulation de charge selon l'une des revendications précédentes, dans lesquelles le rapport du monomère hydrosoluble au monomère liposoluble formant le copolymère est compris entre 70:30 et 99:1 en poids.

6. Procédé de polymérisation en dispersion pour fabriquer des particules de résine de régulation de charge pour un toner électrophotographique selon la revendication 1, dans lequel au moins un monomère hydrosoluble possédant un groupe anionique de type sulfonique, carboxylique ou phosphorique et au moins un monomère liposoluble sont dispersés et polymérisés dans un milieu aqueux contenant de l'eau et un solvant organique miscible à l'eau en présence d'un stabilisant de dispersion et d'un agent de transfert de chaîne, et
le copolymère obtenu constitué par le monomère hydrosoluble et le monomère liposoluble est recueilli sous forme de particules, la polymérisation comprenant les étapes consistant:
- à former un noyau par réaction du monomère liposoluble et du monomère hydrosoluble; et
- à faire croître le noyau ainsi formé;
la température étant plus élevée dans l'étape de croissance du noyau que dans l'étape de formation du noyau.

7. Procédé pour fabriquer des particules de résine de régulation de charge selon la revendication 6, dans lequel le rapport de mélange de l'eau et du solvant organique miscible à l'eau dans le milieu aqueux est compris entre 40:60 et 5:95 en poids.

8. Procédé pour fabriquer des particules de résine de régulation de charge selon les revendications 6 ou 7, dans lequel la température est de 60 à 80°C dans l'étape de formation du noyau et de 70 à 90°C dans l'étape de croissance du noyau.
